

T. C. REDFERN.

SHOE SOLE.

APPLICATION FILED JUNE 16, 1916.

1,255,107.

Patented Jan. 29, 1918.



Fig. 1.



Fig. 2.



Fig. 3.

Thomas Crompton Redfern  
Inventor  
by Lamer Lamer  
Attorney

# UNITED STATES PATENT OFFICE.

THOMAS CROMPTON REDFERN, OF HYDE, ENGLAND.

## SHOE-SOLE.

1,255.107.

Specification of Letters Patent. Patented Jan. 29, 1918.

Application filed June 16, 1916. Serial No. 104,005.

*To all whom it may concern:*

Be it known that I, THOMAS CROMPTON REDFERN, a subject of the King of Great Britain, and resident of Hyde, in the county 5 of Chester, England, have invented certain new and useful Improvements in Shoe-Soles, of which the following is a specification.

This invention relates to the manufacture 10 of soles for boots and shoes from mixtures containing fibrous materials.

If mixtures of fibrous material and india-rubber, gutta-percha and the like are prepared and vulcanized, and if such material is used for making shoe soles, the soles are liable to crack across at the place where the maximum bending occurs, particularly if the material has been rolled out so that the fibers are in the main transverse to the sole. One contributory cause of this cracking is 20 also that the material is liable to expand where the bending occurs, and ultimately some air becomes imprisoned between the composition sole and the middle sole of the shoe, this air tending to stretch the material 25 and to "balloon" it by the constant action of walking.

This difficulty is overcome in the improved article forming the subject of the present application which has all the necessary flexibility and excellent wearing qualities. The fibrous material may consist for instance of disintegrated rubber backing material from worn-out motor tires, or any other comparatively inexpensive fibrous material with 35 some waste rubber if required, and with a comparatively small proportion of india-rubber or gutta-percha and hardening or vulcanizing agents. This material is rolled out into sheets, the rolling being always effected in one direction so that the fibers lie mainly longitudinally to the sheet. The risk 40 of cracking in the shoe soles is eliminated partly by building up the material for the sole in layers placed successively so that the fibers in some layers lie transversely to the fibers in the other layers, and partly by embedding a layer of canvas in the sole near to the upper or inner surface thereof so as to resist stretching at this surface. Experiments 45 have shown that a five-ply sole gives excellent results; the sheets of fibrous material having the fibers running principally in one direction, are rolled out to a thickness about one-fifth of the ultimate thickness 55 required for the shoe soles, and the sheets

so formed are cut into squares which are laid so that the fibers are in one direction in one square and in a cross direction in the next square. In the first, third and fifth layers the fibers are in one direction, and in 60 the second and fourth they are in the other direction. The soles are cut from this sheet so that the fibers lie across the sole in the first, third and fifth layers, while they only lie longitudinally in the second and fourth 65 layers. The cutting is effected in the usual way by knives or dies in a press, the material so cut being laid in the molds. The top layer which will form the upper or inner surface of the sole when vulcanized, is lifted 70 up in the mold, a piece of canvas cut to the required shape is inserted, and the top layer is laid down again. Then the material is vulcanized by heating in molds, preferably under high pressure so that in the finished 75 article the canvas is embedded in the sole between the first and second layers thereof. The canvas is preferably cut so that its edge comes say a quarter of an inch from the edge of the sole everywhere except at the 80 rear part or waist where the sole is chamfered off, but at that part the canvas may come right up to the edge of the material. The object of cutting the canvas so that it shall not come up to the edges in the other 85 parts of the sole is to prevent canvas showing around the edges and to leave them with a good finished appearance.

The sole made up and vulcanized as described above is quite sufficiently flexible for 90 all purposes, while the crossing of the fibers, and the insertion of the layer of canvas absolutely prevents the cracking and stretching of the sole so that "ballooning" cannot occur. Such a sole can be cemented on to 95 the middle sole or welt of a boot and will adhere permanently thereto over the whole surface during wear, or of course it can be stitched or riveted to the middle sole or welt.

The soles may be made up both for fitting to new boots wherein the waist portion extends back into the heel, and also for repairing purposes when the waist portion is chamfered off. The soles are molded to any 105 desired curvature suitable for fitting directly to the insole and to present the desired formation on the wearing surface.

In the accompanying drawing Figure 1 is a plan view of a shoe sole made up for re- 110

pairing purposes, and Fig. 2 is a side view thereof, while Fig. 3 shows a cross section on the line 3—3 of Fig. 1.

- In Fig. 1 the top layer *a* of the fibrous material is shown turned back at the tip to expose the insertion *b* of canvas. In the sectional view Fig. 3 the top layer *a* is the one which is cemented to the middle sole or welt of the boot, and directly beneath this is the insertion of canvas *b*, while *c*, *d*, *e* and *f* are the remaining layers of the fibrous material. In the layers *a*, *d* and *f* the fibers run transversely to the sole, while in the layers *c* and *e* they run longitudinally for example.
- 15 The invention is not limited to the making of soles of five-ply material with the canvas inserted beneath the top layer exactly as above set forth, although experiments seem to indicate that this is the best construction. Any desired number of layers may be used, and in some cases there may be two layers together with the fibers lying the same way therein according to the result which it is desired to attain. The embedding

of the canvas in the material near to the upper surface is a matter of vital importance however, as is also the use of some layers of the material with the fibers lying transversely to the fibers in other layers. The fibers need not necessarily lie exactly transversely and longitudinally in the respective layers, but they may lie somewhat diagonally while still attaining the desired result. The canvas insertion may also be of any shape or size according to requirements.

Having thus described my invention what I claim as new and desire to secure by Letters Patent is:—

As an article of manufacture, a shoe sole consisting of a number of layers of fibrous material disposed with the fibers in one layer lying substantially transversely to the fibers in another, and a layer of canvas inserted between the upper layer of fibrous material and the next layer, the whole being vulcanized together under pressure.

THOMAS CROMPTON REDFERN.